



US007354685B2

(12) **United States Patent**  
**Wu et al.**

(10) **Patent No.:** **US 7,354,685 B2**  
(45) **Date of Patent:** **Apr. 8, 2008**

(54) **PHOTOCONDUCTIVE IMAGING MEMBERS**

(75) Inventors: **Jin Wu**, Webster, NY (US); **Liang-Bih Lin**, Webster, NY (US); **James M. Duff**, Mississauga (CA); **Timothy P. Bender**, Port Credit (CA)

(73) Assignee: **Xerox Corporation**, Norwalk, CT (US)

(\*) Notice: Subject to any disclaimer, the term of this patent is extended or adjusted under 35 U.S.C. 154(b) by 498 days.

(21) Appl. No.: **11/043,716**

(22) Filed: **Jan. 26, 2005**

(65) **Prior Publication Data**

US 2006/0166116 A1 Jul. 27, 2006

(51) **Int. Cl.**

**G03G 15/02** (2006.01)

(52) **U.S. Cl.** ..... **430/58.65**; **430/58.05**;  
..... **430/59.6**; **430/96**

(58) **Field of Classification Search** ..... **430/59.6**,  
..... **430/58.65**, **58.05**, **96**

See application file for complete search history.

(56) **References Cited**

## U.S. PATENT DOCUMENTS

3,121,006 A 2/1964 Middleton et al. ..... 96/1  
3,871,882 A 3/1975 Wiedemann ..... 96/1.5  
4,265,990 A 5/1981 Stolka et al. ..... 430/59  
4,555,463 A 11/1985 Hor et al. ..... 430/59

|                  |         |                         |          |
|------------------|---------|-------------------------|----------|
| 4,587,189 A      | 5/1986  | Hor et al. ....         | 430/59   |
| 4,921,769 A      | 5/1990  | Yuh et al. ....         | 430/64   |
| 5,473,064 A      | 12/1995 | Mayo et al. ....        | 540/141  |
| 5,521,043 A      | 5/1996  | Listigovers et al. .... | 430/59   |
| 6,015,645 A      | 1/2000  | Murti et al. ....       | 430/59   |
| 6,156,468 A      | 12/2000 | Wehelia et al. ....     | 430/65   |
| 6,177,219 B1     | 1/2001  | Yuh et al. ....         | 430/65   |
| 6,255,027 B1     | 7/2001  | Wehelia et al. ....     | 430/65   |
| 6,287,737 B1     | 9/2001  | Ong et al. ....         | 430/58.8 |
| 6,289,190 B1*    | 9/2001  | Amamiya et al. ....     | 399/174  |
| 2003/0059694 A1* | 3/2003  | Tomiuchi et al. ....    | 430/59.6 |
| 2005/0014080 A1* | 1/2005  | Tong et al. ....        | 430/58.8 |

## OTHER PUBLICATIONS

Jennifer Y. Hwang et al., U.S. Appl. No. 10/369,816 filed Feb. 19, 2003 on Photoconductive Imaging Members, now Publication No. 20040161684.

John S. Chambers et al., U.S. Appl. No. 10/370,186 filed Feb. 19, 2003 on Photoconductive Imaging Members, now Publication No. 20040161683.

Cindy C. Chen et al., U.S. Application No. 10/369,812 filed Feb. 19, 2003 on Photoconductive Imaging Members, now Publication No. 20040161682.

\* cited by examiner

Primary Examiner—Mark A. Chapman

(74) Attorney, Agent, or Firm—E. O. Palazzo

(57) **ABSTRACT**

A photoconductive member comprised of a hole blocking layer, a photogenerating layer, and a charge transport layer comprised of a polymer with a low dielectric constant and a charge transport component.

**35 Claims, No Drawings**

## PHOTOCODUCTIVE IMAGING MEMBERS

## CROSS-REFERENCE TO RELATED APPLICATIONS

There is illustrated in U.S. Pat. No. 6,824,940, filed Feb. 19, 2003, entitled Photoconductive Imaging Members, the disclosure of which is totally incorporated herein by reference, a photoconductive imaging member comprised of a hole blocking layer, a photogenerating layer, a charge transport layer, and thereover an overcoat layer comprised of a polymer with a low, for example about 1 to about 2 dielectric constant and charge transport molecules, and wherein the polymer in the overcoat layer may be a poly(cyclo olefin).

There is illustrated in U.S. Pat. 7,037,631, filed Feb. 19, 2003, entitled Photoconductive Imaging Members, the disclosure of which is totally incorporated herein by reference, a photoconductive imaging member comprised of a supporting substrate, a hole blocking layer thereover, a crosslinked photogenerating layer and a charge transport layer, and wherein the photogenerating layer is comprised of a photogenerating component and a vinyl chloride, allyl glycidyl ether, hydroxy containing polymer.

There is illustrated U.S. Pat. 6,913,863, filed Feb. 19, 2003, entitled Photoconductive Imaging Members, the disclosure of which is totally incorporated herein by reference, a photoconductive imaging member comprised of a hole blocking layer, a photogenerating layer, and a charge transport layer, and wherein the hole blocking layer is comprised of a metal oxide; and a mixture of a phenolic compound and a phenolic resin wherein the phenolic compound contains at least two phenolic groups.

There is illustrated in U.S. Pat. 6,875,548, filed Feb. 19, 2003, entitled Photoconductive Imaging Members, the disclosure of which is totally incorporated herein by reference, a photoconductive imaging member comprised of an optional supporting substrate, a photogenerating layer, and a charge transport layer, and wherein said charge transport layer is comprised of a charge transport component and a polysiloxane.

## RELATED PATENTS

Illustrated in U.S. Pat. No. 6,015,645, the disclosure of which is totally incorporated herein by reference, is a photoconductive imaging member comprised of a supporting substrate, a hole blocking layer, an optional adhesive layer, a photogenerator layer, and a charge transport layer, and wherein the blocking layer is comprised, for example, of a polyhaloalkylstyrene.

Illustrated in U.S. Pat. No. 6,287,737, the disclosure of which is totally incorporated herein by reference, is a photoconductive imaging member comprised of a supporting substrate, a hole blocking layer thereover, a photogenerating layer and a charge transport layer, and wherein the hole blocking layer is comprised of a crosslinked polymer derived from the reaction of a silyl-functionalized hydroxy-alkyl polymer of Formula (I) with an organosilane of Formula (II) and water



-continued

(II)



wherein A, B, D, and F represent the segments of the polymer backbone; E is an electron transporting moiety; X is selected from the group consisting of halide, cyano, alkoxy, acyloxy, and aryloxy; a, b, c, and d are mole fractions of the repeating monomer units such that the sum of a+b+c+d is equal to 1; R is alkyl, substituted alkyl, aryl, or substituted aryl; and R<sup>1</sup>, R<sup>2</sup>, and R<sup>3</sup> are independently selected from the group consisting of alkyl, aryl, alkoxy, aryloxy, halogen, cyano, and amino, subject to the provision that two of R<sup>1</sup>, R<sup>2</sup>, and R<sup>3</sup> are independently selected from the group consisting of alkoxy, aryloxy, acyloxy, and halide.

Illustrated in U.S. Pat. No. 5,473,064, the disclosure of which is totally incorporated herein by reference, is a process for the preparation of hydroxygallium phthalocyanine Type V, essentially free of chlorine, whereby a pigment precursor Type I chlorogallium phthalocyanine is prepared by reaction of gallium chloride in a solvent, such as N-methylpyrrolidone, present in an amount of from about 10 parts to about 100 parts, and preferably about 19 parts with 1,3-diiminoisoindolene (DI<sup>3</sup>) in an amount of from about 1 part to about 10 parts, and preferably about 4 parts DI<sup>3</sup>, for each part of gallium chloride that is reacted; hydrolyzing the pigment precursor chlorogallium phthalocyanine Type I by standard methods, for example acid pasting, whereby the pigment precursor is dissolved in concentrated sulfuric acid and then reprecipitated in a solvent, such as water, or a dilute ammonia solution, for example from about 10 to about 15 percent; and subsequently treating the resulting hydrolyzed pigment hydroxygallium phthalocyanine Type I with a solvent, such as N,N-dimethylformamide, present in an amount of from about 1 volume part to about 50 volume parts, and preferably about 15 volume parts for each weight part of pigment hydroxygallium phthalocyanine that is used by, for example, ballmilling the Type I hydroxygallium phthalocyanine pigment in the presence of spherical glass beads, approximately 1 millimeter to 5 millimeters in diameter, at room temperature, about 25° C., for a period of from about 12 hours to about 1 week, and preferably about 24 hours.

Illustrated in U.S. Pat. No. 5,521,043, the disclosure of which is totally incorporated herein by reference, are photoconductive imaging members comprised of a supporting substrate, a photogenerating layer of hydroxygallium phthalocyanine, a charge transport layer, a photogenerating layer of BZP perylene, which is preferably a mixture of bisbenzimidazo(2,1-a-1',2'-b)antra(2,1,9-def:6,5,10-d'e'f')diisoquinoline-6,11-dione and bisbenzimidazo(2,1-a:2',1'-a)antra(2,1,9-def:6,5,10-d'e'f')diisoquinoline-10,21-dione, reference U.S. Pat. No. 4,587,189, the disclosure of which is totally incorporated herein by reference; and as a top layer a second charge transport layer.

The appropriate components and processes of the above patents may be selected for the present disclosure in embodiments thereof.

## REFERENCES

Layered photoresponsive imaging members have been described in numerous U.S. patents, such as U.S. Pat. No.

4,265,990, the disclosure of which is totally incorporated herein by reference, wherein there is illustrated an imaging member comprised of a photogenerating layer, and an aryl amine hole transport layer. Examples of photogenerating layer components include trigonal selenium, metal phthalocyanines, vanadyl phthalocyanines, and metal free phthalocyanines. Additionally, there is described in U.S. Pat. No. 3,121,006, the disclosure of which is totally incorporated herein by reference, a composite xerographic photoconductive member comprised of finely divided particles of a photoconductive inorganic compound dispersed in an electrically insulating organic resin binder.

The uses of perylene pigments as photoconductive substances are also known. There is thus described in Hoechst European Patent Publication 0040402, DE3019326, filed May 21, 1980, the use of N,N'-disubstituted perylene-3,4,9,10-tetracarboxyldiimide pigments as photoconductive substances. Specifically, there is, for example, disclosed in this publication N,N'-bis(3-methoxypropyl)perylene-3,4,9,10-tetracarboxyldiimide dual layered negatively charged photoreceptors with improved spectral response in the wavelength region of 400 to 700 nanometers. A similar disclosure is presented in Ernst Gunther Schlosser, *Journal of Applied Photographic Engineering*, Vol. 4, No. 3, page 118 (1978). There are also disclosed in U.S. Pat. No. 3,871,882, the disclosure of which is totally incorporated herein by reference, photoconductive substances comprised of specific perylene-3,4,9,10-tetracarboxylic acid derivative dyestuffs. In accordance with this patent, the photoconductive layer is preferably formed by vapor depositing the dyestuff in a vacuum. Also, there are disclosed in this patent dual layer photoreceptors with perylene-3,4,9,10-tetracarboxylic acid diimide derivatives, which have spectral response in the wavelength region of from 400 to 600 nanometers. Further, in U.S. Pat. No. 4,555,463, the disclosure of which is totally incorporated herein by reference, there is illustrated a layered imaging member with a chloroiridium phthalocyanine photogenerating layer. In U.S. Pat. No. 4,587,189, the disclosure of which is totally incorporated herein by reference, there is illustrated a layered imaging member with, for example, a perylene, pigment photogenerating component. Both of the aforementioned patents disclose an aryl amine component, such as N,N'-diphenyl-N,N'-bis(3-methyl phenyl)-1,1'-biphenyl-4,4'-diamine dispersed in a polycarbonate binder as a hole transport layer. The above components, such as the photogenerating compounds and the aryl amine charge transport, can be selected for the imaging members of the present disclosure in embodiments thereof.

In U.S. Pat. No. 4,921,769, the disclosure of which is totally incorporated herein by reference, there are illustrated photoconductive imaging members with blocking layers of certain polyurethanes.

Illustrated in U.S. Pat. Nos. 6,255,027; 6,177,219, and 6,156,468, the disclosures of which are totally incorporated herein by reference, are, for example, photoreceptors containing a hole blocking layer of a plurality of light scattering particles dispersed in a binder, reference for example, Example I of U.S. Pat. No. 6,156,468, the disclosure of which is totally incorporated herein by reference, and wherein there is illustrated a hole blocking layer of titanium dioxide dispersed in a specific linear phenolic binder of VARCUM<sup>TM</sup>, available from OxyChem Company.

## BACKGROUND

Disclosed herein are imaging members, and more specifically, single and multi-layered photoconductive imaging

members with a hole blocking or undercoat layer (UCL), a photogenerating layer, a charge transport layer containing a component with a low dielectric constant, such as from about equal to or less than about 2.5, and more specifically, a dielectric constant of from about 1 to about 2.5, and yet more specifically, from about 1.5 to about 2.3.

More specifically, the charge transport layer of the imaging members of the present disclosure are comprised of a polymeric component with a low dielectric constant, examples of this component being poly(phenylene ether) (PPE), poly(cyclo olefin) (PCO), polyesters, polyamides, fluorinated polymers, and polyolefins with no ring structures present on the main polymeric chain, and charge transport molecules. The weight ratio of the polymer and charge transport molecules can be, for example, from about 30/70 to about 80/20. The low dielectric polymer in embodiments possesses a glass transition temperature of from about 80° C. to about 260° C. (degrees Centigrade throughout). Specific examples of PPE polymers are VESTORAN 1900<sup>TM</sup>, a poly-2,6-dimethyl-1,4-phenylene ether polymer, available from Degussa, (temperature of deflection at 0.45 MPa load equal to 185° C. as determined with the known ASTM D648 testing method, and a dielectric constant equal to 2 as determined with the known ASTM D150 at 1 MHz testing method), NORPEX AX290 PPE<sup>TM</sup>, available from Ebbtide Polymers Corporation (temperature of deflection at 1.8 MPa equal to 143° C. as determined with the known ASTM D648 testing method, and a dielectric constant equal to 2 as determined with the known ASTM D150 at 1 MHz testing method). Specific examples of poly(cyclo olefin) polymers include ZEONOR 1600<sup>TM</sup>, a polydicyclopentadiene polymer, available from Zeon Corporation (glass transition temperature equal to 163° C. as determined by DSC; dielectric constant equal to 2.3 as determined with ASTM D150 at 1 MHz), and ZEONEX E48R<sup>TM</sup>, a polydicyclopentadiene polymer, available from Zeon Corporation (glass transition temperature equal to 140° C. as determined by DSC; dielectric constant equal to 2.3 as determined with the ASTM D150 at 1 MHz testing method). Examples of polyesters include EASTAR AN004<sup>TM</sup>, a poly(cyclohexylenedimethylene terephthalate) copolyester, available from Eastman Chemical (temperature of deflection at 0.45 MPa load equal to 103° C. as determined with the ASTM D648 testing method; dielectric constant equal to 2.1 as determined with the ASTM D150 at 1 MHz testing method); examples of polyamides include VESTAMIDE L1940<sup>TM</sup>, a Nylon 12, available from Creanova Inc. (temperature of deflection at 0.45 MPa load equal to 110° C. as determined with the ASTM D648 testing method; dielectric constant equal to 2 as determined with the ASTM D150 at 1 MHz testing method); examples of fluorinated polymers include DuPont 4100 FEP<sup>TM</sup>, a fluorinated ethylene propylene polymer (melting temperature equal to 259° C.; dielectric constant equal to 2 as determined with the ASTM D150 at 1 MHz testing method); examples of polyolefins with no ring structures on the main polymeric chain include VESTYRON 325<sup>TM</sup>, a polystyrene, available from Creanova Inc. (glass transition temperature equal to 89° C. as determined with DSC; dielectric constant equal to 2 as determined with ASTM D150 at 1 MHz testing method), and NOVOLEN 1102J<sup>TM</sup>, a polypropylene, available from BASF (Viscat softening temperature equal to 92° C.; dielectric constant equal to 2.3 as determined with the ASTM D150 at 1 MHz testing method). The thickness of the charge transport layer in embodiments can be, for example, from about 5 microns to about 60 microns, more specifically from about 10

microns to about 40 microns, and yet more specifically from about 15 microns to about 30 microns.

In embodiments the hole blocking layer in contact with the supporting substrate can be situated between the supporting substrate and the photogenerating layer, which is comprised, for example, of the photogenerating pigments of U.S. Pat. No. 5,482,811, the disclosure of which is totally incorporated herein by reference, especially Type V hydroxygallium phthalocyanine, and generally metal free phthalocyanines, metal phthalocyanines, perylenes, titanyl phthalocyanines, selenium, selenium alloys, azo pigments, squaraines, and the like. The imaging members of the present disclosure in embodiments exhibit excellent cyclic/ environmental stability, significantly improved BCR wear resistance and substantially no adverse changes in their performance over extended time periods since, for example, the imaging members comprise a mechanically robust and solvent resistant hole blocking layer, enabling the coating of a subsequent photogenerating layer thereon without structural damage. The photoresponsive, or photoconductive imaging members can be negatively charged when the photogenerating layers are situated between the hole transport layer and the hole blocking layer deposited on the substrate.

Processes of imaging, especially xerographic imaging and printing, including digital, are also encompassed by the present disclosure. More specifically, the layered photoconductive imaging members of the present disclosure can be selected for a number of different known imaging and printing processes including, for example, electrophotographic imaging processes, especially xerographic imaging and printing processes wherein charged latent images are rendered visible with toner compositions of an appropriate charge polarity. The imaging members are in embodiments sensitive in the wavelength region of, for example, from about 500 to about 900 nanometers, and in particular from about 650 to about 850 nanometers, thus diode lasers can be selected as the light source. Moreover, the imaging members of this invention are useful in color xerographic applications, particularly high-speed color copying and printing processes.

## SUMMARY

It is a feature of the present disclosure to provide imaging members with many of the advantages illustrated herein, such as preventing, or minimizing dark injection, a reduction in transit time, and wherein the resulting photoconducting members possess, for example, excellent photoinduced discharge characteristics, cyclic and environmental stability and acceptable charge deficient spot levels arising from dark injection of charge carriers. Furthermore, there are disclosed herein photoconductive imaging members with excellent wear resistance and hardness; acceptable electrical characteristics and the like, and in embodiments improvements in some of these characteristics as compared to a photoconductive member that contains certain polycarbonates as the binder for the charge transport layer.

It is another feature of the present disclosure to provide a charge transport layer with a dielectric constant of less than about 3.

Another feature of the present disclosure is to provide a photoconductor with intrinsic improved wear characteristics and a longer wear life.

Another feature of the present disclosure relates to the provision of layered photoresponsive imaging members,

which are responsive to near infrared radiation of from about 700 to about 900 nanometers.

It is yet another feature of the present disclosure to provide layered photoresponsive imaging members with sensitivity to visible light.

Moreover, another feature of the present disclosure relates to the provision of layered photoresponsive imaging members with mechanically robust and solvent resistant hole blocking layers containing certain phenolic resin binders.

10 In a further feature of the present disclosure there are provided imaging members containing a hole blocking layer comprised of titanium oxide and a phenolic compound/ phenolic resin blend, or a low molecular weight phenolic resin/phenolic resin blend, and which phenolic compound 15 contains at least two, and more specifically, two to ten phenolic groups or low molecular weight phenolic resins with a weight average molecular weight ranging from about 500 to about 2,000, can interact with and consume formaldehyde and other phenolic precursors within the phenolic 20 resin effectively, thereby chemically modifying the curing processes for such resins and permitting, for example, a hole blocking layer with excellent efficient electron transport, and which usually results in a desirable lower residual potential and  $V_{low}$ .

25 Moreover, in another feature of the present disclosure there is provided a hole blocking layer comprised of titanium oxide, a phenolic resin/phenolic compound(s) blend or phenolic resin(s)/phenolic resin blend comprised of a first linear, or a first nonlinear phenolic resin and a second 30 phenolic resin or phenolic compounds containing at least about 2, such as about 2, about 2 to about 12, about 2 to about 10, about 3 to about 8, about 4 to about 7, and the like, phenolic groups, and which blocking layer is applied to a drum of, for example, aluminum and cured at a high 35 temperature of, for example, from about 135° C. to about 165° C.

Aspects of the present disclosure relate to a photoconductive member comprised of a hole blocking layer, a photogenerating layer, a charge transport layer comprised of 40 a polymer with a low dielectric constant, and charge transport molecules; a photoconductive member comprised of a hole blocking layer, a photogenerating layer, and a charge transport layer comprised of a polymer with a low dielectric constant and a charge transport component; a member 45 comprised of a photogenerating layer, and a charge transport layer comprised of a poly(cyclo olefin) polymer and a charge transport component; a member comprised of a supporting substrate, a photogenerating layer, a charge transport layer comprised of a polymer and a charge transport component, 50 and wherein said polymer possesses a suitable dielectric constant; an imaging member wherein the weight ratio of the polymer and charge transport molecules is from about 30/70 to about 80/20, or from about 40/60 to about 60/40, and the like; an imaging member wherein low is equal to or less than 55 about 2.5; an imaging member wherein low is from about 1 to about 2; an imaging member wherein low is 2; an imaging member wherein the polymer present in the charge transport layer is a poly(cyclo olefin); an imaging member wherein the polymer is a poly(phenylene ether); an imaging member 60 wherein the polymer is a poly(cyclohexylenedimethylene terephthalate); an imaging member wherein the polymer (low dielectric polymer) is the poly(cyclo olefin) polymer of a polydicyclopentadiene; an imaging member wherein the polymer is the poly(phenylene ether) polymer of a poly-2, 65 6-dimethyl-1,4-phenylene ether; an imaging member wherein the polymer is a fluorinated ethylene propylene polymer; an imaging member wherein the polymer is a

poly[imino(1-oxododecamethylene)]; an imaging member wherein the polymer is a polystyrene; an imaging member wherein the polymer is a polypropylene; an imaging member wherein the charge transport molecules are selected from the group consisting of low dipole moment arylamine molecules wherein  $\log P$  is equal to or less than about 0 to about 10; an imaging member wherein the charge transport molecules are comprised of bis(3,4-dimethylphenyl)-4-n-butylphenyl amine; an imaging member wherein the charge transport molecules are comprised of bis(3,4-dimethylphenyl)-4-sec-butylphenyl amine; an imaging member wherein the charge transport molecules are comprised of bis(3,4-dimethylphenyl)-4-t-butylphenyl amine; an imaging member wherein the charge transport molecules are comprised of bis(4-t-butylphenyl)-3,4-dimethylphenyl amine; an imaging member wherein the charge transport molecules are comprised of 1,1-bis(di-4-tolylaminophenyl)-4-tert-butylcyclohexane; an imaging member wherein the polymer (present in the top or second charge transport layer) possesses a glass transition temperature of from about 80° C. to about 260° C.; an imaging member wherein the binder polymer possesses a glass transition temperature of from about 160° C. to about 190° C.; an imaging member wherein the hole blocking layer is comprised of a mixture of a metal oxide and a phenolic resin; an imaging member wherein the metal oxide is a titanium oxide; an imaging member wherein the phenolic resin is selected from the group consisting of a formaldehyde polymer generated with phenol, p-tert-butylphenol and cresol; a formaldehyde polymer generated with ammonia, cresol and phenol; a formaldehyde polymer generated with 4,4'-(1-methylallylidene) bisphenol; a formaldehyde polymer generated with cresol and phenol; and a formaldehyde polymer generated with phenol and p-tert-butylphenol; an imaging member wherein the hole blocking layer is of a thickness of about 0.01 to about 30 microns; an imaging member wherein the hole blocking layer is of a thickness of from about 0.1 to about 8 microns; an imaging member further containing an adhesive layer; an imaging member wherein the adhesive layer is comprised of a polyester with an  $M_w$  of about 45,000 to about 75,000, and an  $M_n$  of from about 30,000 to about 40,000; an imaging member further containing a supporting substrate comprised of a conductive metal substrate of aluminum, aluminized polyethylene terephthalate or titanized polyethylene terephthalate; an imaging member wherein the photogenerator layer is of a thickness of from about 0.05 to about 10 microns, and wherein the transport layer is of a thickness of from about 10 to about 50 microns; an imaging member wherein the photogenerating layer is comprised of a photogenerating pigment or photogenerating pigments dispersed in a resinous binder, and wherein the pigment or pigments are present in an amount of from about 5 percent by weight to about 95 percent by weight, and wherein the resinous binder is selected from the group comprised of vinyl chloride/vinyl acetate copolymers, polyesters, polyvinyl butyrals, polycarbonates, polystyrene-b-polyvinyl pyridine, and polyvinyl formals; a member wherein the charge transport layer comprises aryl amines, and which aryl amines are of the formula



wherein X is selected from the group consisting of alkyl, alkoxy and halogen; an imaging member wherein alkyl or alkoxy contains from about 1 to about 12 carbon atoms; an imaging member wherein the aryl amine is N,N'-diphenyl-N,N-bis(3-methyl phenyl)-1,1'-biphenyl-4,4'-diamine; a member wherein the photogenerating layer is comprised of metal phthalocyanines, or metal free phthalocyanines; an imaging member wherein the photogenerating layer is comprised of titanyl phthalocyanines, perylenes, or hydroxygallium phthalocyanines; an imaging member wherein the photogenerating layer is comprised of Type V hydroxygallium phthalocyanine; a method of imaging which comprises generating an image, such as a xerographic image, on the imaging member, developing the latent image, and transferring the developed image to a suitable substrate; an imaging member wherein the weight ratio of the polymer and charge transport molecules is from about 60/40 to about 75/25; an imaging member wherein the member comprises in sequence the photogenerating layer, the charge transport layer containing a poly(cyclo olefin) and optionally further containing a hole blocking layer in contact with a supporting substrate and an adhesive layer in contact with the hole blocking layer; a member comprised of a photogenerating layer, and a charge transport layer comprised of a polymer with a low dielectric constant and a charge transport component; a photoconductive imaging member comprised of a supporting substrate, a hole blocking layer thereover, a photogenerating layer, and a charge transport layer with a dielectric constant of from about 1.5 to about 3; a photoconductive imaging member comprised of a supporting substrate, a hole blocking layer thereover, a photogenerating layer and a charge transport layer containing a polymer binder with a dielectric constant of from about 2 to about 2.5, and wherein the hole blocking layer is comprised of a metal oxide dispersed in a blend of a phenolic compound and a phenolic resin, or a blend of two phenolic resins wherein the first resin possesses a weight average molecular weight of from about 500 to about 2,000 and the second resin possesses a weight average molecular weight of from about 2,000 to about 20,000, and a dopant, for example, of silicon oxide present in an amount of, for example, from about 2 to about 15 weight percent; or a hole blocking layer comprised of a titanium oxide, a dopant, such as a silicon oxide, a phenolic compound or compounds containing at least two, preferably about 2 to about 10 phenolic groups, such as bisphenol S and/or a phenolic resin having a weight average molecular weight of from about 500 to about 2,000, and a known phenolic resin, reference for example U.S. Pat. No. 6,177,219, the disclosure of which is totally incorporated herein by reference; a photoconductive imaging member wherein the hole blocking layer is of a thickness of about 0.01 to about 30 microns, and more specifically, is of a thickness of about 0.1 to about 8 microns; a photoconductive

imaging member wherein the supporting substrate is comprised of a conductive substrate, such as a metal substrate; a photoconductive imaging member wherein the conductive substrate is aluminum, aluminized polyethylene terephthalate, titanized polyethylene, and the like; a photoconductive imaging member wherein the photogenerator layer is of a thickness of from about 0.05 to about 12 microns; a photoconductive imaging member wherein the charge, such as a hole transport layer, is of a thickness of from about 10 to about 50 microns; a photoconductive imaging member wherein the photogenerating layer is comprised of photo-generating pigments dispersed in an optional resinous binder in an amount of from about 5 percent by weight to about 95 percent by weight; a photoconductive imaging member wherein the photogenerating resinous binder is selected from the group consisting of copolymers of vinyl chloride, vinyl acetate and hydroxy and/or acid containing monomers, polyesters, polyvinyl butyrls, polycarbonates, polystyrene-b-polyvinyl pyridine, and polyvinyl formals; a photoconductive imaging member wherein the charge transport layer comprises aryl amine molecules; a photoconductive imaging member wherein the polymer binder is a poly(cyclo olefin), and dispersed therein a charge transport aryl amine of, for example, the formula



wherein X is selected from the group consisting of alkyl and halogen, and wherein the aryl amine is dispersed in a resinous binder; a photoconductive imaging member wherein the aryl amine alkyl is methyl or ethyl, and wherein halogen is chloride or bromide; a photoconductive imaging member wherein the aryl amine is N,N'-diphenyl-N,N-bis(3-methyl phenyl)-1,1'-biphenyl-4,4'-diamine, and related diamines; a photoconductive imaging member wherein the photogenerating layer is comprised of metal phthalocyanines, or metal free phthalocyanines, and the like; a photoconductive imaging member wherein the photogenerating layer is comprised of titanyl phthalocyanines, perylenes, alkylhydroxygallium phthalocyanines, hydroxygallium phthalocyanines, or mixtures thereof; a photoconductive imaging member wherein the photogenerating layer is comprised of Type V hydroxygallium phthalocyanine; a method of imaging which comprises generating an electrostatic latent image on the imaging member illustrated herein, developing the latent image, transferring the developed electrostatic image to a suitable substrate, and fixing the image; a photoconductive imaging member comprised of a hole blocking layer, a photogenerating layer, and a charge transport layer containing aryl amine components and a polymer binder with a suitable dielectric constant, and wherein the hole blocking layer is comprised of a metal oxide; an imaging member wherein the hole blocking layer phenolic compound is bisphenol S, 4,4'-sulfonyldiphenol; an

imaging member wherein the phenolic compound is bisphenol A, 4,4'-isopropylidenediphenol; an imaging member wherein the phenolic compound is bisphenol E, 4,4'-ethylidenebisphenol; an imaging member wherein the phenolic compound is bisphenol F, bis(4-hydroxyphenyl)methane; an imaging member wherein the phenolic compound is bisphenol M, 4,4'-(1,3-phenylenediisopropylidene) bisphenol; an imaging member wherein the phenolic compound is bisphenol P, 4,4'-(1,4-phenylenediisopropylidene)bisphenol; an imaging member wherein the phenolic compound is bisphenol Z, 4,4'-cyclohexylidenebisphenol; an imaging member wherein the phenolic compound is hexafluorobisphenol A, 4,4'-(hexafluoroisopropylidene)diphenol; an imaging member wherein the phenolic compound is resorcinol, 1,3-benzenediol; an imaging member wherein the phenolic compound is hydroxyquinone, 1,4-benzenediol; an imaging member wherein the phenolic compound is of the formula



an imaging member wherein the phenolic resin is selected from the group consisting of a formaldehyde polymer generated with phenol, p-tert-butylphenol and cresol; a formaldehyde polymer generated with ammonia, cresol and phenol; a formaldehyde polymer generated with 4,4'-(1-methylethylidene)bisphenol; a formaldehyde polymer generated with cresol and phenol; and a formaldehyde polymer generated with phenol and p-tert-butylphenol; an imaging member comprised in sequence of a supporting substrate, a hole blocking layer, an optional adhesive layer, a photogenerating layer, and dispersed in a suitable dielectric constant poly(cyclo olefin) binder hole transport components; an imaging member wherein the adhesive layer is comprised of a polyester with an  $M_w$  of about 45,000 to about 75,000, and an  $M_n$  of from about 30,000 to about 40,000; an imaging member wherein the photogenerator layer is of a thickness of from about 0.05 to about 7 microns, and wherein the transport layer is of a thickness of from about 10 to about 55 microns; an imaging member wherein the photogenerating layer is comprised of photogenerating pigments dispersed in a resinous binder, which pigments are selected in an amount of from about 10 percent by weight to about 90 percent by weight, and optionally wherein the resinous binder is selected from the group comprised of vinyl chloride/vinyl acetate copolymers, polyesters, polyvinyl butyrls, polycarbonates, polystyrene-b-polyvinyl pyridine, and polyvinyl formals; an imaging member wherein the charge transport layer comprises suitable known or future developed components, and more specifically hole transport aryl amines, and which aryl amines are of the formula

11



wherein X is selected from the group consisting of aryl, 15  
alkoxy, alkyl and halogen, and the like; an imaging member  
wherein the photogenerating layer is comprised of a hydrox-  
y gallium phthalocyanine; a method of imaging which  
comprises generating an electrostatic latent image on the imaging  
member illustrated herein, developing the latent image  
with a known toner, and transferring the developed electro-  
static image to a suitable substrate like paper. 20

Examples of the charge transport layer components, 25  
which layer in embodiments is of a thickness, for example,  
of from about 10 to about 60, more specifically from about  
15 to about 40, and yet more specifically from about 20 to  
about 30 microns, in contact with the photogenerating layer, 30  
include a low dielectric constant ( $\epsilon < 2.5$ ) polymer and a  
charge transport molecule, or charge transport molecule  
mixtures with a weight ratio of polymer to charge transport,  
for example from about 30/70 to about 80/20, more specifically  
from about 50/50 to about 50/50, and yet more 35  
specifically from about 60/40 to about 40/60. Polymer  
examples are as illustrated herein, and more specifically,  
include amorphous poly(phenylene ethers), available from  
Creanova Inc. as VESTORAN 1900 PPE<sup>TM</sup> with a glass  
transition temperature,  $T_g$ , of 190° C. and a dielectric 40  
constant of 2; poly(cyclo olefins) PCOs available from Zeon  
Chemical as ZEONOR 1600<sup>TM</sup>, with a  $T_g$  of 163° C. and a  
dielectric constant of 2.27; heat resistant poly(cyclohexy-  
lenedimethylene terephthalates) PCTs available from East- 45  
man Chemical as EASTAR AN004<sup>TM</sup>; copolymers with a  
temperature of deflection greater than 103° C. and a dielec-  
tric constant of 2.1; Nylon 12 available from Creanova Inc.  
as VESTAMIDE L1940<sup>TM</sup> with a temperature of deflection  
equal to 110° C. and a dielectric constant equal to 2; 50  
fluorinated polymers available from E.I. DuPont Company  
as 4100 FEPT<sup>TM</sup>, a fluorinated ethylene propylene polymer  
with a melting temperature equal to 259° C. and a dielectric  
constant equal to 2; fluorinated polymers available from E.I. DuPont Company 55  
as 4100 FEPT<sup>TM</sup>, a fluorinated ethylene propylene polymer  
with a melting temperature equal to 259° C. and a dielectric  
constant equal to 2; fluorinated polymers available from E.I. DuPont Company  
as 4100 FEPT<sup>TM</sup>, a fluorinated ethylene propylene polymer  
with a melting temperature equal to 259° C. and a dielectric  
constant equal to 2; polystyrene available from Creanova 60  
Inc. as VESTYRON 325<sup>TM</sup> with a glass transition tempera-  
ture equal to 89° C. and a dielectric constant equal to 2, and  
polypropylene available from BASF as NOVOLEN<sup>TM</sup> with  
a Viscat softening temperature equal to 92° C. and a dielec-  
tric constant equal to 2.3. Examples of the charge transport  
molecules are Ad-11 [bis(3,4-dimethylphenyl)-4-n-bu- 65  
tylphenyl amine], Ad-1 [bis(3,4-dimethylphenyl)-4-sec-bu-  
tylphenyl amine], Ae-22 [bis(3,4-dimethylphenyl)-4-t-bu-  
tylphenyl amine], Ae-25 [bis(4-t-butylphenyl)-3,4-  
dimethylphenyl amine], tert-butyl TAPC [1,1-bis(di-4-  
tolylaminophenyl)-4-tert-butylcyclohexane], of Formulas 1,  
2, 3, 4 and 5, and the like. 70

The selection of a specific charge transport molecule is  
determined by the compatibility with, for example, the  
polymer binder, and the solvents that are used to dissolve the  
charge transport molecules, such molecules including those  
of the formulas 75

12



Ae-25

-continued



Examples of solvents are aromatic hydrocarbons, aliphatic hydrocarbons, halogenated hydrocarbons, ethers, amides and the like, or mixtures thereof. Specific solvent examples are cyclohexanone, cyclohexane, chlorobenzene, carbon tetrachloride, chloroform, methylene chloride, trichloroethylene, tetrahydrofuran, dioxane, dimethyl formamide, dimethyl acetamide and the like, and which solvents can be selected in various amounts, such as from about 50 milliliters to about 1,000 milliliters, or from about 200 milliliters to about 600 milliliters, and the like.

The hole blocking or undercoat layers for the imaging members of the present disclosure contain a number of components including known hole blocking components, such as silanes, doped metal oxides, a metal oxide like titanium, chromium, zinc, tin and the like, a mixture of phenolic compounds and a phenolic resin or a mixture of 2 phenolic resins, and optionally a dopant such as  $\text{SiO}_2$ . The phenolic compounds contain at least two phenol groups, such as bisphenol A (4,4'-isopropylidenediphenol), E (4,4'-ethylidenebisphenol), F (bis(4-hydroxyphenyl)methane), M (4,4'-(1,3-phenylene)diisopropylidene)bisphenol), P (4,4'-(1,4-phenylene)diisopropylidene)bisphenol), S (4,4'-sulfonyldiphenol), and Z (4,4'-cyclohexylidene)bisphenol); hexafluorobisphenol A (4,4'-(hexafluoro isopropylidene)diphenol), resorcinol; hydroxyquinone, catechin, and the like.

The hole blocking layer can be, for example, comprised of from about 20 weight percent to about 80 weight percent, more specifically, from about 55 weight percent to about 65 weight percent of a metal oxide, such as  $\text{TiO}_2$ ; from about 20 weight percent to about 70 weight percent, more specifically, from about 25 weight percent to about 50 weight percent of a phenolic resin; from about 2 weight percent to about 20 weight percent, more specifically, from about 5 weight percent to about 15 weight percent of a phenolic compound preferably containing at least two phenolic groups, such as bisphenol S; and from about 2 weight percent to about 15 weight percent, more specifically, from about 4 weight percent to about 10 weight percent of a plywood suppression dopant, such as  $\text{SiO}_2$ . The hole blocking layer coating dispersion can, for example, be prepared as follows. The metal oxide/phenolic resin dispersion is first prepared by ball milling or dynomilling until the median particle size of the metal oxide in the dispersion is less than about 100 nanometers, for example from about 50 to about

90. To the above dispersion, a phenolic compound and dopant are added followed by mixing. The hole blocking layer coating dispersion can be applied by dip coating or web coating, and the layer can be thermally cured after 5 coating. The hole blocking layer resulting is, for example, of a thickness of from about 0.01 micron to about 30 microns, and more specifically, from about 0.1 micron to about 8 microns. Examples of phenolic resins include formaldehyde polymers with phenol, p-tert-butylphenol, cresol, such as 10 VARCUM™ 29159 and 29101 (OxyChem Company) and DURITE™ 97 (Borden Chemical), formaldehyde polymers with ammonia, cresol and phenol, such as VARCUM™ 29112 (OxyChem Company), formaldehyde polymers with 4,4'-(1-methylethylidene)bisphenol, such as VARCUM™ 15 29108 and 29116 (OxyChem Company), formaldehyde polymers with cresol and phenol, such as VARCUM™ 29457 (OxyChem Company), DURITE™ SD-423A, SD-422A (Borden Chemical), or formaldehyde polymers with phenol and p-tert-butylphenol, such as DURITE™ 20 ESD 556C (Borden Chemical).

Illustrative examples of substrates are as illustrated herein, and specifically layers selected for the imaging members of the present disclosure, and which substrates can be opaque or substantially transparent, comprise a layer of insulating material including inorganic or organic polymeric materials, such as MYLAR® a commercially available polymer, MYLAR® containing titanium, a layer of an organic or inorganic material having a semiconductive surface layer, such as indium tin oxide, or aluminum arranged thereon, or a conductive material inclusive of aluminum, chromium, nickel, brass or the like. The substrate may be flexible, seamless, or rigid, and may have a number of many different configurations, such as for example, a plate, a cylindrical drum, a scroll, an endless flexible belt, and the like. In embodiments, the substrate is in the form of a seamless flexible belt. In some situations, it may be desirable to coat on the back of the substrate, particularly when the substrate is a flexible organic polymeric material, an anticurl layer, such as for example polycarbonate materials commercially available as MAKROLON®.

The thickness of the substrate layer depends on many factors, including economical considerations, thus this layer may be of substantial thickness, for example over 3,000 microns, or of minimum thickness providing there are no significant adverse effects on the member. In embodiments, the thickness of this layer is from about 75 microns to about 300 microns, or from about 100 microns to about 125 microns.

The photogenerating layer, which can, for example, be 50 comprised of hydroxygallium phthalocyanine Type V, is in embodiments comprised of, for example, about 60 weight percent of Type V and about 40 weight percent of a resin binder like polyvinylchloride vinylacetate copolymer such as VMCH (Dow Chemical). The photogenerating layer can 55 contain known photogenerating pigments, such as metal phthalocyanines, metal free phthalocyanines, alkylhydroxyl gallium phthalocyanine, hydroxygallium phthalocyanines, perylenes, especially bis(benzimidazo)perylene, titanyl phthalocyanines, and the like, and more specifically, vanadyl 60 phthalocyanines, Type V hydroxygallium phthalocyanines, and inorganic components such as selenium, selenium alloys, and trigonal selenium. The photogenerating pigment can be dispersed in a resin binder similar to the resin binders selected for the charge transport layer, or alternatively no 65 resin binder is present. Generally, the thickness of the photogenerator layer depends on a number of factors, including the thicknesses of the other layers and the amount

15

of photogenerator material contained in the photogenerating layers. Accordingly, this layer can be of a thickness of, for example, from about 0.05 micron to about 10 microns, and more specifically, from about 0.25 micron to about 2 microns when, for example, the photogenerator compositions are present in an amount of from about 30 to about 75 percent by volume. The maximum thickness of this layer in embodiments is dependent primarily upon factors, such as photosensitivity, electrical properties and mechanical considerations. The photogenerating layer binder resin present in various suitable amounts, for example from about 1 to about 50, and more specifically, from about 1 to about 10 weight percent, may be selected from a number of known polymers such as poly(vinyl butyral), poly(vinyl carbazole), polyesters, polycarbonates, poly(vinyl chloride), polyacrylates and methacrylates, copolymers of vinyl chloride and vinyl acetate, phenolic resins, polyurethanes, poly(vinyl alcohol), polyacrylonitrile, polystyrene, and the like. It is desirable to select a coating solvent that does not substantially disturb or adversely affect the other previously coated layers of the device. Examples of solvents that can be selected for use as coating solvents for the photogenerator layers are ketones, alcohols, aromatic hydrocarbons, halogenated aliphatic hydrocarbons, ethers, amines, amides, esters, and the like. Specific examples are cyclohexanone, acetone, methyl ethyl ketone, methanol, ethanol, butanol, amyl alcohol, toluene, xylene, chlorobenzene, carbon tetrachloride, chloroform, methylene chloride, trichloroethylene, tetrahydrofuran, dioxane, diethyl ether, dimethyl formamide, dimethyl acetamide, butyl acetate, ethyl acetate, methoxyethyl acetate, and the like.

The coating of the photogenerator layers in embodiments of the present disclosure can be accomplished with spray, dip or wire-bar methods such that the final dry thickness of the photogenerator layer is, for example, from about 0.01 to about 30 microns, and more specifically, from about 0.1 to about 15 microns after being dried at, for example, about 40° C. to about 150° C. for about 15 to about 90 minutes.

Illustrative examples of polymeric binder materials that can be selected for the photogenerator layer are as indicated herein, and include those polymers as disclosed in U.S. Pat. No. 3,121,006, the disclosure of which is totally incorporated herein by reference. In general, the amount of polymer binder that is utilized in the photogenerator layer is from about 0 to about 95 percent by weight, from about 25 to about 60 percent, or from about 35 to about 50 percent by weight of the photogenerator layer components.

As optional adhesive layers usually in contact with the hole blocking layer, there can be selected various known substances inclusive of polyesters, polyamides, poly(vinyl butyral), poly(vinyl alcohol), polyurethane and polyacrylonitrile. This layer is, for example, of a thickness of from about 0.001 micron to about 1 micron. Optionally, this layer may contain effective suitable amounts, for example from about 1 to about 10 weight percent, of conductive and nonconductive particles, such as zinc oxide, titanium dioxide, silicon nitride, carbon black, and the like, to provide, for example, in embodiments of the present disclosure further desirable electrical and optical properties.

The charge transport layer can contain a number of known components that, for example, transport holes, examples of which are aryl amines, and which charge transport layer generally is of a thickness of from about 5 microns to about 75 microns, and more specifically, of a thickness of from about 10 microns to about 40 microns, specific examples of

16

transport components include molecules of the following formula dispersed in a low dielectric polymer, such as a poly(cyclo olefin) binder



wherein X is an alkyl group, an alkoxy, an aryl, a halogen, or mixtures thereof, especially those substituents selected from the group consisting of Cl and CH<sub>3</sub>.

Examples of specific aryl amines are N,N'-diphenyl-N, N'-bis(alkylphenyl)-1,1-biphenyl-4,4'-diamine wherein alkyl is selected from the group consisting of methyl, ethyl, propyl, butyl, hexyl, and the like; and N,N'-diphenyl-N,N'-bis(halophenyl)-1,1'-biphenyl-4,4'-diamine wherein the halo substituent is preferably a chloro substituent. Other known charge transport layer molecules can be selected, reference for example, U.S. Pat. Nos. 4,921,773 and 4,464,450, the disclosures of which are totally incorporated herein by reference.

Also included within the scope of the present disclosure are methods of imaging and printing with the photoresponsive devices illustrated herein. These methods generally involve the formation of an electrostatic latent image on the imaging member, followed by developing the image with a toner composition comprised, for example, of thermoplastic resin, colorant, such as pigment, charge additive, and surface additives, reference U.S. Pat. Nos. 4,560,635; 4,298,697 and 4,338,390, the disclosures of which are totally incorporated herein by reference, subsequently transferring the image to a suitable substrate, and permanently affixing the image thereto. In those environments wherein the device is to be used in a printing mode, the imaging method involves the same aforementioned sequence with the exception that the exposure step can be accomplished with a laser device or image bar.

45 The following Examples are being submitted to illustrate embodiments of the present disclosure. These Examples are intended to be illustrative only and are not intended to limit the scope of the present disclosure. Also, parts and percentages are by weight unless otherwise indicated. Comparative Examples with polycarbonate binders for the charge transport layer are also provided.

#### EXAMPLE I

55 Photoreceptor devices (P/R devices) or imaging members were fabricated with the following architectures in the sequence from bottom to top: undercoat or hole blocking layer, photogenerating layer, and charge transport layer containing a component with a dielectric constant of less than about 3, such as 2.3.

60 The undercoat layer was prepared as follows. A titanium oxide/phenolic resin dispersion was prepared by ball milling for 5 days 15 grams of titanium dioxide (STR60NTM, Sakai Company), 20 grams of the phenolic resin (VARCUMTM 29159, OxyChem Company, M<sub>w</sub> of about 3,600, viscosity of about 200 cps) in 7.5 grams of 1-butanol, and 7.5 grams of xylene with 120 grams of 1 millimeter diameter sized ZrO<sub>2</sub>

beads. Separately, a slurry of  $\text{SiO}_2$  and a phenolic resin was prepared by adding 10 grams of  $\text{SiO}_2$  (P100, Esprit) and 3 grams of the above phenolic resin into 19.5 grams of 1-butanol and 19.5 grams of xylene. The resulting titanium dioxide dispersion was filtered with a 20 micrometer pore size nylon cloth, and then the filtrate was measured with Horiba Capa 700 Particle Size Analyzer, and there was obtained a median  $\text{TiO}_2$  particle size of 50 nanometers in diameter and a  $\text{TiO}_2$  particle surface area of  $30 \text{ m}^2/\text{gram}$  with reference to the above  $\text{TiO}_2$ /VARCUM<sup>TM</sup> dispersion. Additional solvents of 5 grams of 1-butanol, and 5 grams of xylene; 2.6 grams of bisphenol S (4,4'-sulfonyldiphenol), and 5.4 grams of the above prepared  $\text{SiO}_2$ /VARCUM<sup>TM</sup> slurry were added to 50 grams of the above resulting titanium dioxide/VARCUM<sup>TM</sup> dispersion, referred to as the coating dispersion. A 30 millimeters in diameter and 340 millimeters in length aluminum pipe cleaned with detergent and rinsed with deionized water was dip coated with the coating dispersion at a pull rate of 160 millimeters/minute, and subsequently, dried at 160° C. for 15 minutes, which resulted in an undercoat layer (UCL) comprised of  $\text{TiO}_2$ /  $\text{SiO}_2$ /VARCUM<sup>TM</sup>/bisphenol S with a weight ratio of about 52.7/3.6/34.5/9.2 and a thickness of 3.5 microns.

A 0.5 micron thick photogenerating layer was subsequently coated on top of the above generated undercoat layer from a dispersion of chlorogallium phthalocyanine Type B (3 parts), and a vinyl chloride/vinyl acetate copolymer, VMCH<sup>TM</sup> ( $M_w$  equal to 27,000, about 86 weight percent of vinyl chloride, about 13 weight percent of vinyl acetate and about 1 weight percent of maleic acid) available from Dow Chemical (2 parts), in 95 grams of toluene/n-butylacetate with a weight ratio of 2 to 1.

The low dielectric constant charge transport layer was prepared as follows. The charge transport solution was ring coated on top of the CGL (charge generating layer), and which solution was comprised of the cyclo(polyolefin) ZEONOR 1600<sup>TM</sup> (Zeon Chemicals,  $T_g$  equal to 163° C.,  $\epsilon$  equal to 2.3), and hole transport molecule of [bis(3,4-dimethylphenyl)-4-sec-butylphenyl amine] with a weight ratio of 75/25 in cyclohexane, and with a solid content of about 20 weight percent. The charge transport layer was dried at 120° C. for 30 minutes resulting in a charge transport thickness of about 25 microns.

A comparative photoreceptor was prepared by repeating the above except that a conventional polycarbonate was selected as the binder in place of the poly(cyclo olefin) for the charge transport layer. A 25  $\mu\text{m}$  thick charge transport layer (CTL/SMTL) was coated on top of the photogenerating layer from a solution of N,N'-diphenyl-N,N'-bis(3-methyl phenyl)-1,1'-biphenyl-4,4'-diamine (8.8 parts) and the known polycarbonate, PCZ-400 [poly(4,4'-dihydroxy-diphenyl-1-1-cyclohexane,  $M_w$  equal to 40,000)] available from Mitsubishi Gas Chemical Company, Ltd. (13.2 parts) in a mixture of 55 grams of tetrahydrofuran (THF) and 23.5 grams of toluene. The CTL was dried at 120° C. for 45 minutes.

The above devices were electrically tested with an electrical scanner set to obtain photoinduced discharge cycles, sequenced at one charge-erase cycle followed by one charge-expose-erase cycle, wherein the light intensity was incrementally increased with cycling to produce a series of photoinduced discharge characteristic curves from which the photosensitivity and surface potentials at various exposure intensities were measured. Additional electrical characteristics were obtained by a series of charge-erase cycles with incrementing surface potential to generate several voltage versus charge density curves. The scanner was equipped

with a scorotron set to a constant voltage charging at various surface potentials. The devices were tested at surface potentials of 500 volts with the exposure light intensity incrementally increased by means of regulating a series of neutral density filters; the exposure light source was a 780 nanometer light emitting diode. The xerographic simulation was completed in an environmentally controlled light tight chamber at ambient conditions (40 percent relative humidity and 22° C.). The following table summarizes the electrical performance for these devices.

| Device                | $V_{low}$ of<br>4.26 erg/cm <sup>2</sup><br>Exposure<br>Energy and<br>166 ms Charge<br>to Exposure<br>Delay (V) | $dV/dX$ | Dielectric<br>Thickness | $V_{depletion}$<br>(V) |
|-----------------------|-----------------------------------------------------------------------------------------------------------------|---------|-------------------------|------------------------|
| Poly(cyclo olefin) CT | 90                                                                                                              | 150     | 10.5                    | 10                     |
| Polycarbonate CT      | 80                                                                                                              | 160     | 8.3                     | 40                     |

$V_{low}$  is the surface potential of the device subsequent to a certain light exposure at a certain time delay after exposure;  $dV/dX$  is the initial slope of the PIDC curve and is a measurement of sensitivity; and  $V_{depletion}$  is linearly extrapolated from the surface potential versus charge density relation of the devices, and is a measurement of voltage leak during charging. Compared with the above known conventional polycarbonate CT (charge transport layer), the above low  $\epsilon$  CT device with the poly(cyclo olefin) exhibits comparable sensitivity,  $V_{low}$ . However, it possesses a higher dielectric thickness than the conventional CT device.

The wear rate of the above devices was tested with a BCR (biased charging roll) wear fixture. The wear rate of the device with the poly(cyclo olefin) was estimated to be about 50 nanometers/kcycle, which is significantly smaller than that of the control or comparative device containing the above PCZ polycarbonate in the charge transport layer (~90 nanometers/kcycle).

## EXAMPLE II

This Example relates to the generation of belt photoreceptors.

Aluminized polyethylene terephthalate substrates were used, on top of which a silane blocking layer (BLS) was coated in glove box at a humidity of less than about 30 percent, for example 27 percent, using 0.0005" Bird Bar. The BLS was prepared by mixing distilled water (5 parts) and 3-aminopropyl triethoxysilane (1 part) for 4 hours, and then adding acetic acid (0.3 part), ethanol (78.7 parts) and heptane (20 parts) in sequence every 10 minutes. The BLS was dried at 120° C. for 1 minute, and the final coating thickness was estimated to be about 50 nanometers.

An adhesive interface layer (IFL), comprised of a polyester with a  $M_w$  of about 49,000 in THF/cyclohexanone (70/30 weight/weight), was then coated on top of the BLS in a protective hood with 0.0005" Bird bar. The IFL was dried at 120° C. for 1 minute, and the final coating thickness was estimated to be about 50 nanometers.

A charge generator layer (BGL, binder generator layer) was then coated on top of the IFL in the above hood with a 0.00025" Bird Bar. The BGL was prepared by roll milling a mixture of hydroxygallium phthalocyanine (Type V, 1.33 parts), polystyrene-co-poly(vinyl pyridine) (ASVP1811, 1.5

19

parts), toluene (44.33 parts), and stainless steel shot at 200 rpm for 20 hours. The BGL was dried at 120° C. for 1 minute, and the final coating thickness was estimated to be about 0.4 micron, and which coating had an optical density of from about 0.8 to about 1 at 670 nanometers.

A small molecule transport layer (SMTL) was then coated on top of the above BGL in a glove box with 6" wide, 10 mil Bird Bar to 25 microns in thickness. The SMTL was dried at ambient conditions for about 3 to about 5 minutes, and then at 135° C. for 10 minutes. The SMTL was prepared by dissolving NORPEX AX 290 PPETM (Ebbtide Polymers Corporation, temperature of deflection equal to 143° C.,  $\epsilon$  equal to 2), and hole transporting components of [bis(3,4-dimethylphenyl)-4-n-butylphenyl amine] with a weight ratio of 70/30 in chlorobenzene.

It is believed that the photoreceptor of the above Example II will possess a number of the desirable characteristics as recited herein.

The claims, as originally presented and as they may be amended, encompass variations, alternatives, modifications, improvements, equivalents, and substantial equivalents of the embodiments and teachings disclosed herein, including those that are presently unforeseen or unappreciated, and that, for example, may arise from applicants/patentees and others.

What is claimed is:

1. A photoconductive member comprised of a hole blocking layer, a photogenerating layer, and a charge transport layer comprised of a polymer with a low dielectric constant and a charge transport component wherein said low dielectric constant is equal to or less than about 2.5.
2. A member in accordance with claim 1 wherein the weight ratio of the polymer and charge transport component is from about 30/70 to about 80/20.
3. A member in accordance with claim 1 wherein said low is less than about 2.5.
4. A member in accordance with claim 1 wherein said low is from about 1 to about 2.
5. A member in accordance with claim 1 wherein said low is 2.
6. A member in accordance with claim 1 wherein said polymer is a poly(cyclo olefin).
7. A member in accordance with claim 1 wherein said polymer is a poly(cyclohexylenedimethylene terephthalate).
8. A member in accordance with claim 1 wherein said polymer is the poly(cyclo olefin) polymer of a polydicyclopentadiene.
9. A member in accordance with claim 1 wherein said polymer is the poly(phenylene ether) polymer of a poly-2, 6-dimethyl-1,4-phenylene ether.
10. A member in accordance with claim 1 wherein said polymer is a fluorinated ethylene propylene polymer, a poly[imino(1-oxododecamethylene)], a polystyrene, or a polypropylene.
11. A member in accordance with claim 1 wherein said charge transport component is comprised of molecules selected from the group consisting of low dipole moment arylamine molecules wherein said low is equal to or less than about 0 to about 3.
12. A member in accordance with claim 1 wherein said charge transport component is comprised of molecules of bis(3,4-dimethylphenyl)-4-n-butylphenyl amine.
13. A member in accordance with claim 1 wherein said charge transport component is comprised of molecules of bis(3,4-dimethylphenyl)-4-sec-butylphenyl amine, bis(3,4-dimethylphenyl)-4-t-butylphenyl amine, bis(4-t-butylphe-

20

nyl)-3,4-dimethylphenyl amine, or 1,1-bis(di-4-tolylaminophenyl)-4-tert-butylcyclohexane.

14. A member in accordance with claim 1 wherein said polymer possesses a glass transition temperature of from about 80° C. to about 260° C.

15. A member in accordance with claim 1 wherein said polymer possesses a glass transition temperature of from about 160° C. to about 190° C.

16. A member in accordance with claim 1 wherein said 10 hole blocking layer is comprised of a mixture of a metal oxide and a phenolic resin.

17. A member in accordance with claim 16 wherein said metal oxide is a titanium oxide.

18. A member in accordance with claim 16 wherein said 15 phenolic resin is selected from the group consisting of a formaldehyde polymer generated with phenol, p-tert-butylphenol and cresol; a formaldehyde polymer generated with ammonia, cresol and phenol; a formaldehyde polymer generated with 4,4'-(1-methylethylidene) bisphenol; a formaldehyde polymer generated with cresol and phenol; and a formaldehyde polymer generated with phenol and p-tert-butylphenol.

19. A member in accordance with claim 1 wherein said 20 hole blocking layer is of a thickness of from about 0.01 to about 30 microns.

20. A member in accordance with claim 1 wherein said 25 hole blocking layer is of a thickness of from about 0.1 to about 8 microns.

21. A member in accordance with claim 1 further containing an adhesive layer.

22. An imaging member in accordance with claim 21 wherein the adhesive layer is comprised of a polyester with an  $M_w$  of about 45,000 to about 75,000, and an  $M_n$  of from about 30,000 to about 40,000.

23. A member in accordance with claim 1 further containing a supporting substrate comprised of a conductive metal substrate of aluminum, aluminized polyethylene terephthalate or titanized polyethylene terephthalate.

24. A member in accordance with claim 1 wherein said 40 photogenerator layer is of a thickness of from about 0.05 to about 10 microns, and wherein said transport layer is of a thickness of from about 10 to about 50 microns.

25. A member in accordance with claim 1 wherein said photogenerating layer is comprised of a photogenerating pigment or photogenerating pigments optionally dispersed in a resinous binder, and wherein said pigment or pigments are present in an amount of from about 5 percent by weight to about 95 percent by weight, and wherein the resinous binder is selected from the group comprised of vinyl chloride/vinyl acetate copolymers, polyesters, polyvinyl butyral, polycarbonates, polystyrene-*b*-polyvinyl pyridines, and polyvinyl formals.

26. A member in accordance with claim 1 wherein said 55 charge transport component is comprised of aryl amine molecules, and which aryl amines are of the formula



**21**

wherein X is selected from the group consisting of alkyl, alkoxy and halogen.

**27.** A member in accordance with claim **26** wherein alkyl contains from about 1 to about 10 carbon atoms.

**28.** A member in accordance with claim **26** wherein the aryl amine is N,N'-diphenyl-N,N-bis(3-methyl phenyl)-1,1'-biphenyl-4,4'-diamine, and wherein the photogenerating layer is comprised of metal phthalocyanines, or metal free phthalocyanines.

**29.** A member in accordance with claim **1** wherein said photogenerating layer is comprised of titanyl phthalocyanines, perylenes, or hydroxygallium phthalocyanines.

**30.** A member in accordance with claim **1** further containing a protective overcoating layer.

**31.** A member in accordance with claim **1** wherein the weight ratio of the polymer and charge transport molecules is from about 60/40 to about 75/25.

**32.** A member in accordance with claim **1** wherein said member comprises in sequence said photogenerating layer, said polymer and said charge transport layer, and said hole

**22**

blocking layer in contact with a supporting substrate, and an adhesive layer in contact with the hole blocking layer, and wherein said polymer is a poly(cyclo olefin).

**33.** A method of imaging which comprises generating an image on the member of claim **1**, developing the image, and optionally transferring the developed image to a suitable substrate.

**34.** A photoconductor comprised of a photogenerating layer, and a charge transport layer comprised of a poly(cyclo olefin) polymer and a charge transport component, and wherein said polymer possesses a dielectric constant of equal to or less than 2.5.

**35.** A photoconductor comprised of a supporting substrate, a photogenerating layer, a charge transport layer comprised of a polymer and a charge transport component, and wherein said polymer possesses a dielectric constant of less than 2.5.

\* \* \* \* \*